

May 17, 1960

T. HINDLE ET AL

2,936,796

PAPER-MAKERS' DRYER FELT

Filed July 3, 1956

2 Sheets-Sheet 1



Fig. 1

DACRON      DACRON + COTTON

COTTON      ASBESTOS + NYLON

ASBESTOS      NYLON + COTTON

NYLON      DACRON + NYLON

ASBESTOS + COTTON



Fig. 2



Fig. 5



Fig. 6



Fig. 7



Fig. 8



Fig. 9

Inventors  
Thomas Hindle  
Edward Race  
by Thomas Hindle  
Atty's

May 17, 1960

T. HINDLE ET AL  
PAPER-MAKERS' DRYER FELT

2,936,796

Filed July 3, 1956

2 Sheets-Sheet 2



Fig. 3



Fig. 4

Inventors  
Thomas Hindle  
Edward Race  
by *Thomas Hindle & Edward Race*  
Atty's

2,936,796

## PAPER-MAKERS' DRYER FELT

Thomas Hindle and Edward Race, Blackburn, England, assignors to Scapa Dryers Limited, Blackburn, England, a corporation of England

Application July 3, 1956, Serial No. 595,616

16 Claims. (Cl. 139—426)

This invention pertains to paper-makers' dryer "felts," which term is explained below and which are endless bands or belts of woven textile fabric employed for supporting and conveying the paper web delivered by a paper-making machine while the web is moved through a drying zone or zones; the present invention relating more especially to a felt of novel construction having a much longer useful life than felts as heretofore constructed.

Paper-makers' dryer felts are of great length and for use in making certain types of paper may be very wide. Such felts must be woven by the use of special looms and because of their size and thickness, great quantities of yarn are used in their construction, so that the total cost of such a felt to the paper manufacturer is substantial, often running into many thousands of dollars. On the other hand, such felts are subjected during use to very exacting conditions, being called upon to run without intermission for twenty-four hours a day; to flex rapidly about heated cylindrical drums and felt rolls of relatively small diameter; to withstand the effects of moisture; to withstand the degrading action of certain chemicals which are invariably present in the paper web, and of the abrasive wear and oil contamination to which they may be subjected especially at their marginal portions. At the same time, they must be operative to draw away the moisture from the paper web and rapidly to yield it in liquid form or dissipate it in the form of vapor; to provide a substantially uniform and smooth surface upon which the paper web rests and such as will not impart any appreciable pattern effect, for example of the weave structure, to the wet paper web.

In the early days of paper-making and paper-making machines, these felts were of wool and were subjected to operations during manufacture, which doubtless justified the use of the term "felt" in this connection. However, these wool felts were gradually superseded by cotton, and were at first of single ply cotton duck, but such single ply fabrics were in turn, superseded by multi-ply fabrics which afforded a greater degree of softness and smoothness, which are highly desirable qualities, especially when the felt is to be used in the manufacture of the finer grades of paper. The expression ('ply') is used herein not in its limited sense as regards the construction of weave, but to define layers in which one material predominates compared with another or others, it being obvious that there must be some migration of such other material or materials from one layer into, at least, one other layer in order to produce homogeneous woven fabric.

Because these all-cotton felts were subjected to high temperatures during the paper-drying process, their useful life was shortened by degradation of the cotton so as to be much shorter than desirable, from the paper-makers' standpoint owing to the high cost of replacing such a felt. Such degradation was assumed to be due to the heat, and in the hope of extending the useful life of the felt, it was proposed to employ asbestos for a part, at least,

of the customary cotton upon the theory that, because of the well-recognized resistance of asbestos to the effects of heat, the length of life of the felt would be increased by the incorporation of asbestos. These so-called "asbestos" felts, which, in fact, were combinations of asbestos and cotton, the latter being employed to provide the requisite tensile strength, have not superseded the all-cotton felts, the choice of the composition (whether wholly cotton or partly cotton and partly asbestos) of the felt being determined by the conditions appertaining on that section of the dryer part of the paper machine to be clothed. In recent years, other materials than wool, cotton and asbestos have been suggested as useful in the manufacture of dryer felts; for example, some of the synthetic fibers such as nylon or Dacron.

Although the use of some of these other materials in the manufacture of dryer felts has been proposed, they have not, as yet, superseded cotton, since cotton does possess certain desirable basic characteristics for use in such felts. For example, it is relatively cheap; it is of high tensile strength; it possesses reasonable abrasion resistance and has a relatively high modulus of elasticity under low load so that it can be made into fabrics of good dimensional stability. On the other hand, from the dryer felt standpoint specifically, cotton has some undesirable characteristics, in particular its poor resistance to heat, especially under moist conditions. Moreover, in the presence of weak acids and/or trace amounts of iron (often encountered in the paper-drying operation), the degradation of cotton in the presence of moisture and heat is greatly accelerated. Furthermore, cotton, as compared with most of the other natural fibers, has poor flexural endurance. As compared with cotton, certain synthetic fibers, notably nylon and Dacron, are superior in strength, abrasion resistance, flexural endurance and heat and acid resistance. In these respects, nylon has the greater abrasion resistance and flexural endurance while on the other hand Dacron is outstandingly superior to nylon in its resistance to heat and in its ability to resist attack by acids at high temperatures.

Thus, it appears that these particular synthetics, nylon or Dacron, might well be used in the manufacture of dryer felts; for instance, by making dryer felts wholly of nylon or Dacron. On the other hand, the initial cost of felts made wholly of nylon or Dacron is much higher than those made wholly of cotton or cotton and asbestos because of the cost of the raw materials employed. Experience has shown that the increased service life of such all-synthetic felts is not always sufficient to justify the substitution of all-synthetic felts for those of the materials heretofore commonly used. Thus, it has been suggested that a practical solution of the problem might be found in using a combination of the synthetic fibers with cotton or cotton and asbestos. It was first suggested that the mere blending of nylon or Dacron staple fiber with cotton would provide a long-wearing dryer felt, but it was soon realized that since cotton fibers are degraded by heat or acid, so that they break into shorter fibers as they are continuously flexed about the rolls of a papermaking machine, the mere incorporation of a small percentage of synthetic fibers would not greatly retard the disintegration of the cotton yarns. Further experiment showed that desirable results could be obtained by twisting continuous filament yarns of synthetic material with cotton yarns in such a manner that the filament yarns would form open helical wrappings around a core of cotton, and that if the pitch of the synthetic helix is not greater than half the length of the individual cotton fibers, the yarn will tend to maintain its integrity even though the individual cotton fibers sustain considerable degradation, and it was found that by incorporating not more than 12½% of the synthetic material, representing a cost in-

crease of only 15% or 16%, as compared with all-cotton felt, the increase in the life of the felt was far in excess of that required to compensate for the added cost of manufacture. Such a fabric is more fully disclosed in the patent to Hindle and Hall, No. 2,882,933, dated April 21, 1959.

As above noted, the incorporation of asbestos yarns in a dryer felt has been very widely adopted because the inclusion of the asbestos was supported to impart added resistance to degradation of the felt structure by the action of heat. It is true that asbestos-cotton felts have shown greater dimensional stability and a longer life than the all-cotton felt, but recent experimental investigation appears to indicate that the longer life of the asbestos-cotton felt, as compared with the all-cotton felt, is not due to the fact that asbestos itself is substantially unaffected by heat, but that certain other properties of the asbestos are responsible for the improved results. Customary practice in the use of asbestos in a dryer felt (it being noted that yarns made wholly of asbestos fibers are too weak to be used in the manufacture of a heavy textile fabric) is to blend from 10% to 20% of cotton or other cellulose fiber with the asbestos to assist in the spinning and weaving operations. Even such yarns are relatively weak and it is not uncommon to use asbestos yarn with a cotton core such that the asbestos yarn may contain up to 30% or more of cellulosic fibers, representing up to 90% of the total strength of the yarn. Customarily, the asbestos yarns are so interwoven that they appear on the working face of the felt, that is to say, the face on which the paper web rests, and consequently the cotton component of these composite yarns is fully exposed to the heat and moisture conditions, so that the cotton degrades rapidly and there is a substantial loss of strength. Thus, when the face of the felt consists of asbestos yarns, the ultimate strength of the felt is determined by the degree to which the integrity of the back cotton warp yarns is maintained, and thus the cotton yarns in the back of the fabric should be protected so far as possible from the effects of the heat to which the face of the fabric is exposed. At first glance, it might be thought that the asbestos at the face of the fabric would protect the cotton at the back of the felt, but it is a proven fact that asbestos is a poor heat insulator as compared with most other fibrous materials, in spite of the fact that asbestos is commonly employed as an essential component in many insulating fabrics. In the course of investigation, an all-cotton felt was compared with a felt in which all of the filling yarns were asbestos and the warps of the working face of the felt were asbestos (that is to say, asbestos reinforced with cotton), these felts being subjected, at their working faces to a temperature of 350° F. Rather astonishingly, it was found that these asbestos-cotton felts sustained a greater loss in strength than the all-cotton felt and that the loss in strength of the face warp yarns of these asbestos-cotton felt was as great as the loss in strength of the face warp yarns of the cotton felt. Obviously, this was due to the fact that virtually the entire strength of the asbestos face yarns resided in their cotton components. To overcome this loss in strength in the asbestos face yarns, it was proposed to substitute Dacron for the cotton in the composite asbestos yarns, but this arrangement still failed to produce optimum results because asbestos is not a good heat insulator but on the other hand is, in fact, a good conductor of heat as compared with organic fibres, so that the cotton warp yarns of the back of the fabric were still subject to degradation by heat transmitted to them by the asbestos. It was found that in a felt so constructed the yarns in the back of the fabric were degraded from 50% to 100% more than those of an all-cotton felt under similar conditions of treatment.

Apart from degradation by heat and by mechanical causes, there are two agencies which play a major part in the destruction of a papermaker's felt particularly of a

cotton felt or a cotton containing felt, though affecting other materials, including the synthetic materials aforesaid, to a lesser degree. One is acid or even a mildly acid condition and the other is iron in some of its compounds. Thus, the rate of degradation of cotton at 212° F. and a pH value of 4.5 is twenty times that of cotton at 212° F. and a pH value of 6.5. Moreover, in the presence of as little as one part in 10,000 of ferric oxide, cotton at 212° F. and at a pH value of 6.5 is degraded many times more rapidly than iron-free cotton under the same conditions. It thus appears that the major contribution of asbestos to the lengthening of the service life of a dryer felt is its heretofore unrecognized ability to protect the cotton or other component of the felt from degradation by acid and by the hydrolytic decomposition which also affects other material than cotton and is catalyzed by the ever-present traces of iron compounds.

The majority of papers are slightly acid and the acidity of the paper web tends to increase as it passes through the dryer section of the paper-making machine, due to the concentrating of initially very dilute sulphuric acid emanating from the hydrolysis of alum. As the web dries, this sulphuric acid is transferred to the dryer felt, there to accumulate and become more and more concentrated. Thus, it is not unusual for the aqueous extract of a used cotton dryer felt to show a pH value as low as 2.5 and a sulphate content as high as 2.4%. The rate of degradation of cotton at high temperatures increases very rapidly with decrease in pH value and it is believed that acid degradation plays at least as great a part as the heat in the destruction of cotton dryer felts. When asbestos is present in the felt, it shows a preferential absorption of acid, the acid being taken up exclusively by the magnesium oxide component of the asbestos with the formation of water soluble magnesium sulphate. It has also been shown by experiment that the asbestos is capable of rendering any iron compounds harmless to the cotton. Thus, samples of all-cotton felt and an asbestos-cotton felt were treated (every four hours for a period of 48 hours) by alternately wetting them in a solution of an iron salt containing one part in 10,000 of iron and then drying at a temperature of 220° F., while similar samples were treated with iron-free distilled water at the same pH value. The resultant losses in strength were as follows:

|                                                                 | Percent loss in strength |
|-----------------------------------------------------------------|--------------------------|
| An all-cotton felt free from iron                               | 18                       |
| An all-cotton felt containing a small amount of added iron      | 70                       |
| An asbestos-cotton felt free from added iron                    | 23                       |
| An asbestos-cotton felt containing a small amount of added iron | 25                       |

That is, the loss in strength in the presence of iron and absence of asbestos is four times the loss when iron is not present; and, when both asbestos and iron are present, the iron causes no appreciable increase in the rate of degradation of the cotton.

The present invention is based upon the above discoveries and provides a dryer felt which, in respect to cost of production, as compared with increased service life, is wholly practical. Briefly stated, the dryer felt of the present invention consists of textile yarns interwoven to form a multi-ply fabric, said fabric comprising a top or face layer for contact with the paper web, which is predominantly of a material which is a good heat insulator, and which is substantially unaffected by exposure to moisture, to acid, to iron and to the temperatures encountered in the use of a dryer felt; an intermediate layer integrally joined to the top or face layer and underlying the latter, said intermediate layer being predominantly of a material which reacts chemically with the acid and/or iron present in the paper web, so as to neutralize or prevent the degrading effects of acid or iron upon cellulosic fibers comprised in the felt, and a back or bottom layer integrally joined with the intermediate layer,

and which is of a tensile strength comparable to that of cotton and which is capable of accepting all of the moisture passed to it from the face of the felt, and which is capable of readily releasing this moisture as vapor. Preferably, the face layer is of Dacron, a material which can, by capillarity, accept very high quantities of water, but which has such a low moisture regain that it cannot always hold the water it accepts; and, which is virtually unaffected by, but will not absorb either acid or trace quantities of iron. Therefore, the back layer of the felt should be composed of yarns of a material capable of accepting all of the moisture which passes through the felt from its front face and which is capable of readily releasing this moisture in the form of vapor. Cotton has these latter characteristics as well as substantial tensile strength, and is desirable for the back face of the felt. Since Dacron does not absorb acid or trace quantities of iron, it does not protect the cotton back from the effects of these reagents, although it does have high insulating value and thus protects the cotton back from heat degradation. To protect the cotton from the action of acid and iron, the intermediate layer should be of a character such as to absorb the acid and nullify the effects of minute quantities of iron, and asbestos provides these characteristics.

In accordance with the present invention, warp-faced fabrics have been woven comprising two, three or four plies, wherein the exposed surface layer of the face ply consists predominantly of Dacron warp yarns; the back ply warps are of cotton predominantly, preferably reinforced with helically wound synthetic filament yarns, and all of the filling yarns are asbestos yarns which constitute the intermediate layer between the face layer of Dacron and the back layer of cotton. Also, weft-faced fabrics have been woven in which the exposed face weft yarns are of Dacron; the center and back weft yarns are of asbestos and the whole of the warp yarns are of cotton, preferably reinforced with helically-wound synthetic filament yarns. No particular weave structure appears to be necessary to obtain highly desirable results. The expression "asbestos yarns" is used above and hereinafter to mean a yarn made of asbestos fibres suitably reinforced by other fibres, such as cotton.

The superiority in heat resistance of this new type of Dacron-faced, asbestos-cotton filled dryer felt over conventional asbestos-cotton felts may be illustrated by the following example wherein a three-layer felt, according to the present invention, was compared with a conventional asbestos felt of identical weave structure, by subjecting the working face of each of them to the same heat conditions for a given time. Under these circumstances, the conventional asbestos-cotton felt lost 48% of its initial strength, whereas the Dacron-faced felt, according to the present invention, lost 7%. The face warp of the conventional asbestos felt lost 71% of its initial strength whereas the Dacron face warp of the felt of the present invention lost 9%. The cotton back of the asbestos felt lost 55%, while the cotton back of the Dacron-faced felt lost 12%.

In the accompanying drawings, which are wholly diagrammatic—

Fig. 1 is a fragmentary diagrammatic plan view of a section of a paper-makers' dryer felt embodying the present invention;

Fig. 2 is a fragmentary diagrammatic transverse section on the line 2—2 of Fig. 1, illustrative of a felt embodying the essential characteristics of a felt constructed according to the present invention;

Fig. 3 is a diagram illustrative of a weave structure, which gives a substantially warp-faced fabric, such as may be employed in a three-ply felt embodying the invention;

Fig. 4 is a view of the same kind as that of Fig. 3, but illustrating another weave structure which gives a weft-faced fabric.

Figs. 5, 6 and 7 are views similar to Fig. 2 but illustrative of other embodiments of the invention;

Fig. 8 is a side elevation showing a composite yarn comprising asbestos reinforced with cotton; and

Fig. 9 is a view similar to Fig. 8, showing a composite yarn comprising cotton reinforced with nylon.

Referring to Fig. 1, the character B designates the body portion of a felt made according to the present invention; while the characters M designate the marginal portions of the felt and which may, if desired, be of the construction and materials more fully described in the patent to Hall, No. 2,612,190, September 30, 1952, and which provides high resistance, for the marginal portions of the felt, in particular, to the effects of abrasion and exposure to oil. However, this particular marginal construction is optional, with respect to the felt of the present invention.

Referring to Fig. 2, which is a diagrammatic transverse section through the body portion of the felt, and without any attempt to indicate actual weave structure, the numeral 10 designates the exposed face of the top layer of a three-layer fabric, the numeral 11, the intermediate layer, and the numeral 12, the exposed face of the back or rear layer. As illustrated in Fig. 2, the exposed face 25 of layer 10 consists of Dacron combined with a certain percentage of nylon. The relative proportions of nylon and Dacron in this face layer will depend upon the specific conditions to which the felt will be subjected during use. Thus, for example, when excessive moisture is present or there is severe mechanical abrasion, or the felt rolls are of unusually small diameter, the nylon should be in major proportion. On the other hand, when acid 30 conditions lower than pH 4.5 are encountered, or when the felt runs very hot and unusually dry, then the Dacron should be in major proportion.

As illustrated in Fig. 2, the intermediate layer 11 consists of asbestos reinforced with cotton. Thus, it may comprise a yarn consisting of a cotton core 13, Fig. 8, with a wrapping 14 of asbestos roving or the like, or it 40 may consist of any other desirable or usual composite yarn in which asbestos is reinforced in one way or another with a stronger fiber. The back layer 12 of this fabric of Fig. 2 is shown as consisting of cotton yarn reinforced with nylon.

While the arrangement illustrated in Fig. 2 suggests that the asbestos be confined to the intermediate layer 11, it is to be understood that a greater proportion of asbestos may be employed if desired, for example all of the filling yarns of layers 11 and 12 may be of asbestos yarns, or the filler yarns of all three layers may be asbestos.

In Fig. 5, the face layer 10a is shown as consisting wholly of Dacron, while the intermediate layers 11a and the back layer 12a are like those of Fig. 2. In Fig. 6, the face layer 10b is of Dacron; the back layer 12b is of cotton, while the intermediate layer is of asbestos yarn, 55 reinforced with cotton, while in Fig. 7, the face layer 10c is of Dacron, the back layer 12c is of cotton and the intermediate layer 11c is of asbestos yarn.

Referring to Fig. 3, there is shown an actual weave structure of a three-ply, warp-faced woven fabric in which the surface layer of the upper ply 10 is comprised of the warps 1, 2 and 3. The warps 1, 2, and 3 are of Dacron, for example 5s/3 (cotton count) spun Dacron. The warps 4, 5, 6, 7 and 8 are composed of, for example, 65 8s/6 cotton plied with two filament yarns, each of 210 total denier, of nylon. The warps 2 and 3 form stitches integrally uniting the face ply 10 and the intermediate ply 11, while the warps 6 and 7 form stitches which integrally unite the intermediate ply 11 and back ply 12.

In this fabric all of the filler yarns a, b and c are of asbestos; or, more strictly speaking, asbestos spun around a core of 6s cotton or spun nylon to a resultant count of 0.8s. The Dacron warps employed in this structure are highly resistant to degradation by heat or acid and securely bind in the filler yarns a, b and c. The filler

yarns, being of asbestos, act to neutralize the effects of acid and/or iron upon the cotton warps 4, 5, 6, 7 and 8.

In the fabric of Fig. 4, which is also a three-ply fabric, the face layer 10x is comprised of weft yarns, and the whole of the warp is composed of 40 ends per inch of 8s/6 cotton reinforced with two filament nylon yarns each of 210 total denier. The filler yarns *a* are of 5s/3 Dacron. The filler yarns *b* and *c* are of asbestos; for example, asbestos containing 10% to 15% of cotton spun around a core of 20s/3 cotton to a resultant count of 0.8s.

When nylon is employed as a reinforcement for cotton, it is preferable so to combine the cotton and nylon strands that the nylon forms an open helix or helices embracing the cotton as illustrated in Fig. 9, and although the asbestos yarn may consist of an asbestos strand wrapped about a cotton or nylon core, such composite yarn may alternatively itself comprise an asbestos core encased in an open jacket consisting of helical windings of the reinforcing synthetic material.

Since, as above noted, the particular reason for employing the asbestos is to provide a barrier which preferentially absorbs any acid present and neutralizes the latter, and also to protect the cotton yarns from the degrading effect of minute traces of iron, it is contemplated that the proportion of asbestos in the felt may be substantially reduced as compared with the customary amount, without, in any, lessening the service life of the felt. Thus, the asbestos fillers in the bottom and intermediate plies, for example, might be replaced under certain circumstances, with cotton or in particular cotton reinforced with nylon, or with some other suitable organic fibrous material, thus reducing weight and difficulties in manufacture.

When herein reference is made to the face ply of the felt as, for example, "of Dacron" or as "predominantly of Dacron," it is to be understood that this terminology is to be interpreted as meaning that the exposed surface layer, at least, of the said ply is predominantly of Dacron, although the ply itself may also comprise a substantial percentage of yarns of other material, for example, asbestos.

While certain desirable embodiments of the invention have herein been suggested by way of example, it is to be understood that the invention is broadly inclusive of any and all equivalents and modifications coming within the terms of the appended claims.

We claim:

1. A paper-makers' dryer felt consisting of textile yarns interwoven to form a multi-ply fabric, said fabric comprising a top or face layer whose exposed surface, which contacts the paper web, is predominantly of an organic material which is substantially unaffected by exposure to the acids, compounds of iron, or the temperatures encountered in the use of a dryer felt and which is a good heat insulator, an intermediate layer integrally joined to the face layer and underlying the latter, said intermediate layer comprising a material which reacts chemically with acids initially present in the paper to neutralize the same, and a back layer integrally joined to the intermediate layer and which comprises predominantly a material having a tensile strength, moisture absorption and modulus of elasticity similar to those of cotton.

2. A paper-makers' dryer felt according to claim 1 wherein the heat insulating material which forms the exposed surface of the top layer is synthetic material, and the acid neutralizing material of the intermediate layer is asbestos.

3. A paper-makers' dryer felt according to claim 1 wherein the exposed surface of the face layer comprises predominantly Dacron, the rear layer comprises predominantly cotton, and the intermediate layer comprises a material operative to shield the cotton of the rear layer from the effects of acid and/or iron in the paper web.

4. A paper-makers' dryer felt according to claim 3

wherein the warps of the rear layer are predominantly of cotton reinforced with a synthetic filamentous material.

5. A paper-makers' dryer felt according to claim 1 and comprising more than two plies, wherein the exposed surface of the face layer is predominantly of Dacron, the major portions of the warps of intermediate and rear plies are of cotton reinforced with nylon, and the filler yarns of all plies are of asbestos reinforced with an organic filamentous material.

6. A paper-makers' dryer felt according to claim 1 wherein the exposed surface of the face layer is predominantly of Dacron in the form of warp yarns, the exposed surface of the rear layer is formed of warp yarns predominantly of cotton, and the filler yarns in each of the several plies are of asbestos reinforced with an organic filamentous material.

7. A paper-makers' dryer felt according to claim 1 and comprising more than two plies, wherein the face ply is a warp-faced fabric in which the warps are of Dacron, the intermediate layer comprises wefts of asbestos reinforced with cotton, and some, at least, of the Dacron warps of the face layer form stitches at intervals which unite the face and intermediate layers.

8. A paper-makers' dryer felt according to claim 1 wherein the face ply is a weft-faced fabric in which the face wefts are of Dacron, the intermediate and back wefts are of asbestos and all of the warps comprise cotton.

9. A paper-makers' dryer felt according to claim 8 wherein all of the warps are of cotton reinforced with a filamentous material.

10. A paper-makers' dryer felt according to claim 1 wherein the exposed surface of the face layer consists of yarns of a synthetic material which is a heat insulator superior to asbestos and which is substantially inert as respects the action of moisture, high temperature, acid or iron to which the felt is exposed during normal use, the warps of the rear ply are predominantly of cotton, and means interposed between the exposed surface of the front ply and the rear ply which is operative to shield cotton comprised in the rear ply from the action of acid or iron penetrating from the face ply.

11. A paper-makers' dryer felt according to claim 10 wherein the means for shielding the cotton of the rear ply comprises asbestos contained in the filling yarns in certain at least of said plies.

12. A paper-makers' dryer felt consisting of textile yarns interwoven to form a multi-ply fabric, said fabric comprising a face ply, the surface of which contacts the paper when the felt is in use, whose warps are predominantly of Dacron reinforced with nylon, and the wefts which form an intermediate layer are of asbestos reinforced with nylon.

13. A paper-makers' dryer felt consisting of textile yarns interwoven to form a multi-ply fabric, said fabric comprising a face layer, which contacts the paper web when the felt is in use, whose exposed surface is predominantly of a synthetic material which is highly resistant to heat within the range to which the paper-makers' dryer felt is normally exposed, which is a good heat insulator, which is non-absorbent as respects acid or traces of iron commonly present in the paper web, and which is readily capable of transmitting moisture from the paper web to an intermediate layer of the felt, the rear layer of the felt comprising predominantly organic material which is highly absorbent of moisture, and a material within the structure of the felt which is operative to neutralize any acid and to shield the rear layer from the effects of any iron compounds held in suspension or solution in the moisture which is transmitted from the front layer to the rear layer.

14. A paper-makers' dryer felt consisting of textile yarns interwoven to form a multi-ply fabric, the exposed surface of the face layer, which contacts the paper web when the felt is in use, being predominantly of an organic material which is a good heat insulator, certain of the

yarns comprised in the rear layer of the fabric being of cotton, and a layer of moisture-permeable material which reacts between the exposed surface of the face layer and said cotton yarns for shielding the latter from the degrading action of any acid and/or iron compounds to which the felt is exposed during use.

15. A paper-makers' dryer-felt comprising textile yarns interwoven to form a multi-ply fabric, said fabric having a top or face layer whose exposed surface, which contacts the paper web when the felt is in use, is predominantly of an organic fibrous material selected from the group consisting of Dacron and nylon, an intermediate layer integrally joined to the face layer and which comprises asbestos, and a back layer integrally joined to the intermediate layer and which comprises predominantly cotton.

16. A paper-makers' dryer-felt comprising textile yarns

interwoven to form a multi-ply fabric, said fabric having a paper-contacting surface which is predominantly of Dacron, an intermediate layer comprising asbestos and a rear layer comprising predominantly cotton.

References Cited in the file of this patent

UNITED STATES PATENTS

|           |                |               |
|-----------|----------------|---------------|
| 2,152,415 | Krasselt       | Mar. 28, 1939 |
| 2,506,667 | Hall           | May 9, 1950   |
| 2,540,874 | Geddings       | Feb. 6, 1951  |
| 2,542,297 | Sunbury et al. | Feb. 20, 1951 |
| 2,604,689 | Hebeler        | July 29, 1952 |

FOREIGN PATENTS

|               |               |
|---------------|---------------|
| Australia     | Aug. 15, 1949 |
| Great Britain | Oct. 12, 1948 |
| Great Britain | June 9, 1954  |